

Dec. 28, 1948.

E. C. HANDWERK ET AL

2,457,548

PROCESS FOR CONDENSING ZINC VAPOR

Filed June 22, 1946



INVENTOR  
Erwin C. Handwerk  
George T. Mahler  
BY  
Perrine, Edmonds, Morton and Barrows  
ATTORNEYS

## UNITED STATES PATENT OFFICE

2,457,548

## PROCESS FOR CONDENSING ZINC VAPOR

Erwin C. Handwerk and George T. Mahler, Palmerton, Pa., assignors to The New Jersey Zinc Company, New York, N. Y., a corporation of New Jersey

Application June 22, 1946, Serial No. 678,540

2 Claims. (Cl. 75—88)

1

This invention relates to condensing zinc vapor, and has for its object an improved method thereof.

In the customary pyrometallurgical practices of smelting zinc ores, the zinc is recovered as molten metal by condensing the zinc vapor contained in the gaseous products of the smelting operation. In continuously operated smelting equipment, such as modern externally heated retorts or electro-thermally heated retorts, the zinc vapor diluted with ordinary smelting gases, such as carbon monoxide and the like, is passed through a condenser in which an operating temperature is maintained for effective condensation of the zinc vapor to molten zinc. This temperature may advantageously be of the order of from 500 to 550° C. Since the gas frequently enters the condenser at a temperature at least 300° C. higher than the proper operating temperature, it is customary in such cases to thermally associate with the condenser suitable heat-dissipating means for maintaining the proper temperature, and especially is this so with zinc smelting equipment of relatively large capacity. In the copending patent application of ourselves and Harry C. Haupt, Serial No. 626,508, filed November 3, 1945, there is disclosed a splash zinc condenser in which the heat-dissipating means for the condensing chamber are cooling jackets thermally associated with the outside walls of the chamber, and in a companion application Ser. No. 633,004, filed December 5, 1945, we described the positioning of positive artificial cooling means within the condensing chamber itself.

A characteristic feature of the splash condenser described in the aforementioned applications is the provision of a substantial volume of molten zinc in the bottom of the condensing chamber, which is kept under continuous agitation and which communicates with another body of molten zinc in a discharge well exterior of the condensing chamber. While investigating the performance of this splash condenser under commercial operating conditions, we have discovered that it is possible to maintain a proper operating temperature within the condensing chamber by appropriate dissipation of heat from the body of molten metal in the discharge well. Thus, by direct artificial cooling of the molten metal in the discharge well, we have found that sufficient heat can be withdrawn from the communicating body of molten zinc in the condensing chamber to maintain the proper operating temperature of the chamber.

Thus, the method of the present invention com-

2

prises passing a gaseous stream containing zinc vapor through a condensing chamber having a body of molten zinc therein, maintaining exteriorly of the chamber a body of molten zinc communicating with the molten zinc in the chamber, and controlling the operating temperature of the condensing chamber by subjecting the exterior and communicating body of molten zinc to direct artificial cooling while facilitating circulation of molten zinc between the two bodies thereof by agitating the molten zinc in the chamber. Both bodies of molten zinc are of substantial volume, but the volume of the exterior body of molten zinc may be and usually is considerably smaller than that in the condensing chamber. The direct artificial cooling of the exterior body of molten zinc is regulated by the temperature of the molten zinc therein, or in the condensing chamber, to maintain the proper operating temperature of the chamber. The cooling of the exterior and communicating body of molten zinc is advantageously effected by a stream of extraneous cooling medium flowing through a confined path in said molten zinc but out of direct contact therewith. Intimate contact between the zinc vapor bearing gaseous stream and the molten zinc within the condensing chamber is effected by hurling molten zinc from said body thereof upwardly into the upper portion of the chamber through which the gaseous stream passes.

The foregoing and other novel features of the invention will be best understood from the following description taken in conjunction with the accompanying drawing, which illustrates, by way of example, a condenser in which the invention may advantageously be practiced, and in which—

Fig. 1 is a longitudinal sectional elevation of the condenser, and

Fig. 2 is a top plan view of the condenser.

The condenser illustrated in the drawing is of the splash type described in the aforementioned applications, to which reference is made for a fuller description of such features of construction as are not directly concerned with the present invention and hence not herein illustrated and described. As shown in the drawing, the condenser comprises a generally rectangular condensing chamber 5 having a zinc vapor inlet 6 approximate one end and an exhaust or waste gas outlet 7 approximate its other end, and is lined with suitable refractory material. The zinc vapor inlet 6 is connected by a pipe 8 to a source of zinc vapor, such as a vertical zinc smelting retort. The zinc vapor inlet 6 and the gas outlet 7 are shielded by depending refractory baffles 9

and 10, respectively, to prevent splashing or spraying of molten zinc into the inlet or outlet.

The condensing chamber communicates, beneath the lower edge of its end wall 11, with a discharge well 12 having an overflow spout 13 determining the level *a* of the body of molten zinc in the collecting chamber. A collecting trough 14 receives the molten metal overflowing the spout 13 and conveys it to casting equipment or the like. The lower portion of the end wall 11 dips into the molten metal between the condensing chamber and the communicating discharge well and seals the condensing chamber from the atmosphere at this point. The overflow spout 13 and trough 14 may be dispensed with, and molten metal manually dipped or otherwise suitably removed from the well 12 for casting, storage or other purpose. As zinc vapor condenses in the chamber 5, the resulting molten zinc collects in the body of molten zinc in the chamber, and molten zinc is removed from the well 12 by continuous overflow, by dipping at periodic intervals, or in any other suitable manner to maintain, for all practical purposes, a substantially constant volume of molten zinc in the chamber.

A generally cylindrical rotor 15 is mounted within the condensing chamber 5. The rotor is carried by a hollow or axially bored metal shaft 16 mounted in bearings outside the condenser. The shaft 16 is horizontally disposed and extends through the side walls of the condensing chamber between the zinc inlet and the gas outlet in a direction generally transverse to the direction of gas flow through the chamber. The rotor may be constructed of graphite, silicon carbide or other suitable refractory, and is separated from direct contact with the shaft 16 by a sleeve 18 of insulating cement. The shaft 16 has a plurality of circumferentially spaced peripheral ribs 19 embedded in the cement sleeve, and the bore of the rotor has a plurality of spaced recesses 20 filled with the cement of the sleeve, so that the shaft, sleeve and rotor are effectively keyed together. The shaft 16 is cooled by the flow of a cooling medium, such as water, through its axial bore.

The peripheral surface of the rotor 15 has a plurality of circumferentially spaced pockets or cups 21. The pockets have a generally scoop-like section with a relatively long advancing flat section and a shallow semi-circular depression at the inner end or bottom of the pocket. The shaft 16 is positioned at a level substantially above that of the molten zinc adapted to be held in the chamber 5, and the rotor 15 is of such outside diameter that its lowermost pocket is beneath the molten zinc level *a*. The shaft 16 (and hence the rotor 15) is driven by an electric motor or other suitable source of power (not shown).

Artificial cooling means are operatively associated with the discharge well 12 to cool the body of molten zinc therein. While the artificial cooling means may be of any suitable type, satisfactory results are secured with a bayonet water-cooler depending from a suitable support or resting on the refractory floor or bottom of the well. As illustrated in the drawing, a metallic (e. g. iron) cooling shell 22 of substantial width and having water inlet and outlet pipes 23 and 24, respectively, is operatively supported by a frame 25 and depends into and substantially to the bottom of the well 12. Any other suitable cooling liquid may be circulated through the shell 22 instead of water.

In the practice of the invention in the condenser illustrated in the drawing, a continuous

stream of gas containing zinc vapor enters the condensing chamber beneath the baffle 9 of the inlet 6, and flows in a generally horizontal direction through the chamber and beneath the baffle 10 to the exhaust gas outlet 1. Where the entering gas is derived from a vertical retort smelting operation, it will have a temperature of around 820-900° C., and will generally contain around 30 to 50% zinc vapor diluted for the most part with carbon monoxide gas. The rotor 15 is rotated at a relatively high speed, say around 100 to 150 R. P. M., clockwise as viewed in Fig. 1, so that the pockets 21 in rapid succession pick up and throw sheets or showers of molten zinc into the gas stream. The upwardly-directed and rapidly succeeding sheets or showers of molten metal splash into the shower or rain of molten metal particles falling through the chamber, and also splash against the baffle 9 and the roof of the condensing chamber, with the result that the condensing chamber is substantially filled with sheet-like showers and moving particles of molten zinc which form ideal nuclei for the condensation and subsequent coalescence of the zinc vapor.

25 The rotor 15 agitates the body of molten zinc in the bottom of the condensing chamber and the molten metal is hence in constant motion. The temperature of this body of molten zinc may be, for all practical purposes, taken as the operating 30 temperature of the condensing chamber and hence of the condenser itself. In accordance with the invention, this body of molten zinc is maintained at the contemplated operating temperature by the dissipation or withdrawal of heat therefrom into the artificially cooled body of molten zinc in the discharge well. Thus, circulation of the cooling medium in the cooling shell 22 abstracts heat from the molten zinc in the well and as a consequence heat is withdrawn from the communicating molten zinc in the condensing chamber. Due to its agitated condition and its inherent good heat conductivity, the molten zinc in the condensing chamber readily gives up its heat to the artificially cooled communicating 40 molten zinc in the discharge well. By properly controlling the artificial cooling applied to the molten zinc in the well, heat is withdrawn or dissipated from the molten zinc in the condensing chamber in such amount and at such a rate as to maintain the proper operating temperature of the condenser, e. g. 500 to 550° C. At this operating temperature, substantially all of the zinc vapor is condensed, the condensed molten zinc is collected in the body of molten zinc in the condensing chamber, and molten zinc is withdrawn from the chamber into the discharge well.

55 The artificial cooling to which the molten zinc in the well 12 is subjected is advantageously regulated by varying the submerged area of the cooling shell 22. This may be done manually by lifting or lowering the shell, or by varying its inclination. Since the operating temperature of the condenser is indicated by the temperature of the molten zinc in the condensing chamber, the artificial cooling may advantageously be regulated by that temperature as obtained from a suitably positioned pyrometer or other temperature measuring instrument. Due to the agitation of the molten zinc in the condensing chamber, the molten zinc in the communicating well is in constant circulation and when the slight operating temperature differential between the two bodies of molten zinc for a particular condenser has been ascertained, the artificial cooling may be regulated by the temperature of the molten zinc

in the well. The artificial cooling may be automatically adjusted in response to temperature changes of the molten zinc in either the condensing chamber or well. Thus, as shown in the drawing, the submerged area of the cooling shell 22 is automatically regulated by a temperature-responsive actuating means 26 operatively connected to a pyrometer 27 positioned in the molten zinc in the well 12. If the temperature of the molten zinc in the well rises, the actuating means 26, responding to that temperature rise, lowers the shell 22, thereby increasing its submerged area and hence its cooling effect. If, on the other hand, the temperature of the molten zinc decreases, the actuating means 26 raises the shell 22 and thereby decreases its cooling effect. In this manner, the temperature of the molten zinc in the well is maintained within predetermined limits by regulating the cooling effect of the shell 22, and thereby the operating temperature of the condensing chamber is controlled. As previously stated, the pyrometer 27 may be positioned in the molten zinc in the condensing chamber, although it is generally more convenient and equally satisfactory to position it in the molten zinc in the well.

Molten zinc may be manually or otherwise dipped from the discharge well 12, instead of overflowing the spout 13 into the trough 14. Dipping is generally carried out at periodic but frequent intervals, and only such an amount of molten zinc is removed from the well at each dipping as to maintain, for practical purposes, a substantially constant volume of molten zinc in the condensing chamber. A certain minimum volume of molten zinc should be maintained in the well in order to provide an adequate heat reservoir for withdrawing heat from the condensing chamber and dissipating such heat through the artificial cooling means as well as to prevent freezing during such interruptions in condenser operation as occasionally occur in practice, and the depth of molten zinc in the well should be sufficient to permit adequate immersion of the cooling means. In practice, heat is dissipated from the molten zinc in the well at about the same rate that heat is withdrawn from the condensing chamber, and the molten zinc in the well is hence not unduly cooled. While the relative volumes of molten zinc in the condensing chamber and discharge well will depend upon the size and capacity of the condenser, and perhaps to a lesser degree upon the effectiveness of the agitation of the molten zinc in the chamber, the following example is indicative of these factors:

The condenser was of the splash type illustrated in the drawing and had a condensing capacity of about 6 tons of zinc per day of 24 hours. About 2000-2500 pounds of molten zinc was maintained in the condensing chamber and about 500 pounds in the discharge well, and the area of communication between the two bodies of molten zinc was of the order of one-half square foot. The rotor 15 lifted about 5000 pounds of molten zinc per minute. In other words, molten zinc in amount approximately equivalent to the body thereof in the condensing chamber was lifted from that body and thrown into the chamber by the rotor every 30 seconds. This resulted in a vigorous agitation of the molten zinc in the chamber which was transmitted to the communicating body of molten zinc in the well. The operating temperature of the condensing chamber was maintained slightly above 500° C. by im-

mersion of a water-cooled shell 22 in the molten metal in the well 12, the immersion area of the shell (of the order of about one-half square foot) being manually regulated in accordance with the temperature of the molten zinc in the well. With continuous overflow of molten zinc from the discharge well 12 into the trough 14, the temperature of the molten zinc in the well is 10-15° C. lower than that of the molten zinc in the condensing chamber. With manual dipping from the discharge well in the course of which about 1000 pounds of molten zinc is removed from the well and the depth of molten zinc in the condensing chamber drops from about 7 inches to about 5 inches, the temperature difference between the molten zinc in the chamber and well increases from 10-15° C. at the start of dipping to about 50° C. at the termination of dipping. Dipping takes only a few minutes (usually less than 5 minutes) and may conveniently be carried out at two hour intervals.

The external and communicating body of molten zinc need not be held in the discharge well of the condenser, but may be an equivalent externally positioned auxiliary cooling well in similar communication with the condensing chamber, as for example at the opposite end or at the side of the condenser. Aside from the fact that molten zinc is not ordinarily removed from such an auxiliary cooling well, the molten zinc therein is artificially cooled and functions in the same manner as herein described with respect to the molten zinc in the discharge well 12. An adequate depth of molten zinc should be maintained in the well 12 or equivalent cooling well to permit such immersion of the artificially cooling means as is required for the practice of the invention. With a water-cooled iron shell 12, a thin coating or crust of solidified zinc forms on the submerged area of the shell, but this does not adversely affect the cooling efficiency, and moreover protects the iron shell from corrosion by the molten zinc. While it is now our preferred practice to use a cooling shell for the dissipation of heat from the molten zinc in the cooling well, any other appropriate cooling means may be employed. Whenever situated, the area of communication between the condensing chamber and cooling well should be substantial, and preferably as large as practical, while effectively sealing the condensing chamber against the entrance of atmospheric air, in order to provide an adequate area of heat exchange between the communicating bodies of molten zinc and to provide some agitation or circulation of the molten metal in the cooling well in consequence of the agitation of the communicating body of molten zinc in the condensing chamber.

We claim:

1. The method of condensing zinc vapor which comprises passing a gaseous stream containing zinc vapor through a condensing chamber having a body of molten zinc therein, maintaining exteriorly of the condensing chamber a body of molten zinc communicating with the body of molten zinc in the chamber, effecting intimate contact between the gaseous stream and the molten zinc within the condensing chamber by hurling molten zinc from said body thereof upwardly into the upper portion of the condensing chamber through which the gaseous stream passes while facilitating circulation of molten zinc between the bodies thereof by the agitation of the body of molten zinc in the condensing chamber, and controlling the operating tempera-

7  
ture of the condensing chamber by subjecting said exterior and communicating body of molten zinc to the cooling effect of a stream of extraneous cooling medium flowing through a confined path in said molten zinc but out of direct contact therewith.

2. The method of condensing zinc vapor which comprises passing a gaseous stream containing zinc vapor through a condensing chamber having a body of molten zinc in the bottom thereof, withdrawing molten zinc from said body thereof into a communicating body of molten zinc exterior of the chamber to maintain a practically constant volume of molten zinc in the chamber, effecting intimate contact between the gaseous stream and the molten zinc within the condensing chamber by hurling molten zinc from said body thereof upwardly into the upper portion of the condensing chamber through which the gaseous stream passes while facilitating circulation of molten zinc between the bodies thereof by the agitation of the body of molten zinc in the condensing chamber, and controlling the operating temperature of said condensing chamber by subjecting the molten zinc in said exterior and communicating body 25 448. thereof to the cooling effect of a stream of ex-

traneous cooling medium flowing through a confined path in said molten zinc but out of direct contact therewith.

5  
ERWIN C. HANDWERK.  
GEORGE T. MAHLER.

#### REFERENCES CITED

The following references are of record in the file of this patent:

#### 10 UNITED STATES PATENTS

| Number       | Name         | Date          |
|--------------|--------------|---------------|
| 1,871,657    | Bunce        | Aug. 16, 1932 |
| 2,231,023    | Nelson       | Feb. 11, 1941 |
| 15 2,238,819 | Neve         | Apr. 15, 1941 |
| 2,294,546    | Gentil       | Sept. 1, 1942 |
| 2,348,194    | Crane et al. | May 9, 1944   |

#### 15 FOREIGN PATENTS

| Number | Country | Date         |
|--------|---------|--------------|
| 55,473 | Sweden  | May 24, 1922 |

#### 20 OTHER REFERENCES

Chemical Age, November 4, 1944, pp. 447 and 25 448.